

March 2, 1943.

A. J. MORWAY ET AL

2,312,725

GREASE AND MANUFACTURE THEREOF

Filed June 10, 1940



Arnold J. Morway Inventor  
John C. Zimmer  
By J. H. Small Attorney

## UNITED STATES PATENT OFFICE

2,312,725

## GREASE AND MANUFACTURE THEREOF

Arnold J. Morway, Clark Township, Union County, and John C. Zimmer, Union, N. J., assignors to Standard Oil Development Company, a corporation of Delaware

Application June 10, 1940, Serial No. 339,616

14 Claims.

(Cl. 252—39)

This invention relates to a novel type of grease and method of preparing same and more particularly it relates to a new type of lime soap grease having certain novel characteristics and prepared by a certain novel procedure.

Heretofore probably the most common method of preparing lime soap greases has been to heat the required amount of fat and lime together with a small proportion (e. g. 10%) of the oil to be used, to a temperature of about 300° F. to 350° F., cooking the mixture until complete saponification, adding the remaining oil, thereby cooling the mixture to about 210° F. to 225° F., adding 1% to 2% of water to assist in forming the grease structure and then finishing and drawing the product at a temperature between about 200° F. and 180° F. It has also been suggested to dissolve a fatty acid in part of the oil, warming the solution to about 120° F. to 150° F., and then adding a suspension of hydrated lime in the remaining oil, but this process has been confined to greases made of relatively light oils, for instance, having a viscosity of about 40 to 50 seconds Saybolt at 210° F. In the past it has been thought impossible to prepare calcium grease containing high viscosity oils directly, and the only attempt to use such high viscosity oils involved the preparation of the grease from a low viscosity oil (75 seconds Saybolt viscosity at 210° F.) and subsequently blending heavy oils into the resultant finished grease after hydration. It was also necessary to have black or special grease making oils for this type of lubricant and these greases at best were always opaque due to the relatively large amount of water present which was used in preparing the greases and all such greases were buttery in structure, having no tendency to string out. It has been very difficult in the past to make any lime soap grease with a high viscosity oil base stock.

However, the present invention enables the use of high viscosity oils and permits the production of greases of various desired consistencies and at the same time obtains an unexpectedly useful result, namely that the greases prepared do not soften when worked but in fact usually get harder when worked.

The invention comprises broadly mixing together an oil solution of the fatty acid or mixture of fatty acids and an oil suspension of hydrated lime (which may be stabilized by small amounts of lime or soda soap) at a temperature between about 150° F. to 200° F., stirring (if necessary cooling) the mixture and drawing the finished grease at a temperature below about 175° F.,

5 preferably at a temperature not substantially above 160° F. In carrying out this process it is preferred to use only part of the oil during the soap formation step and then to add the remaining part of the oil to assist in cooling or quenching the hot grease mixture. It is also preferred to work and cool the finished product to even a lower temperature than indicated above because in general the further this cooling is carried the more tendency will the finished product have to harden or increase in consistency when it is subsequently worked; for instance, the grease may be made at a temperature of 190° F. but cooled while stirring to 130° F. whereupon the resultant product will have fairly high unworked penetration of about 380 to 400 (A. S. T. M. method) but upon working the penetration will be reduced to about 320 or even below 300. These greases are also transparent. Accordingly, the production of lubricating greases which may vary from a semifluid soft grease or a soft bodied grease which hardens to a solid lubricant on working or dispensing is of special value in automotive chassis lubrication and severe industrial service. The ability of the greases of this invention to harden on working, such as by passing through the usual type grease guns, is of particular advantage in that some garage and filling station equipment requires a lubricant that must flow under its own weight in order to be easily dispensable, but under most conditions greases of this type will not remain on the lubricated parts without drippage, while ordinary greases which are hard when unworked soften considerably on working such as encountered on passage through grease dispensing equipment. This novel grease, due to its unique features, has all the advantages with none of the disadvantages that ordinary greases would have under these conditions.

40 The oil base stock to be used in this invention is preferably a mineral oil fraction having a viscosity of about 55-250 or more seconds Saybolt at 210° F., and preferably having a viscosity of about 70-200 seconds at 210° F. This oil can be either a single fraction or it can be a blend of several different fractions, for instance, a blend of a heavy cylinder oil, a distillate or propane deasphalted residual bright stock having a viscosity of about 200 seconds Saybolt at 210° F. and a minor proportion of a distillate having a viscosity of about 50 seconds Saybolt at 210° F. These oils should preferably be derived from crudes of nonparaffinic type, for instance, preferably oils derived from Coastal or Mid-Continent crudes,

e. g. of naphthenic, asphaltic, aromatic or mixed paraffinic type, although Pennsylvania bright stock or cylinder oils are also suitable for the preparation of these greases.

The fatty acid to be used may be either a single fairly pure fatty acid such as oleic acid, stearic, or palmitic acid, or mixture of the various fatty acids, preferably having more than 10 carbon atoms, such as, for instance, a mixture of fatty acids obtained by the oxidation of paraffin waxes; also fatty acids obtained from animal or vegetable fats or fatty oils may be used such as the fatty acids obtained from lard, tallow, corn oil, palm oil, or from castor oil, cottonseed oil, soya bean oil, etc., or the mixed fatty acids called tall oil fatty acids as obtained from the sulfide paper process, or mixtures of any of these various types of acids may be used.

The lime to be used for neutralizing the fatty acids should preferably be added in the form of hydrated lime and it should be substantially free from any water not chemically combined as  $\text{Ca}(\text{OH})_2$ . Also, it should be substantially free from any particles of unslaked burned lime or carbonated lime. Although it is preferred to use a hydrated lime which is relatively pure calcium hydroxide, a very small amount of magnesium content can be tolerated as in the case of hydrated lime obtained from a technical limestone.

In carrying out the invention the amount of fatty acid to be used should be approximately 2% to 25% by weight of the total raw materials. The amount of lime to be used can be calculated from the saponification number of the fatty acids. Generally, with this procedure the finished product should contain less than about 0.75% of free acid.

Other known addition agents may be added to the greases if desired, such as, for instance, soda, potassium, barium, aluminum, lead, zinc or other grease-making soaps; polybutenes, acryloid derivatives, or other string-imparting linear hydrocarbon, or ester polymers, dyes and oxidation inhibitors, e. g. alpha-naphthyl amine, phenol alpha-naphthyl amine, benzyl penta-amino phenol, guaiacol, or other amines or phenols or phenolic ethers. These oxidation inhibitors may be used in concentration of about .05% to 3.0% and assist in preventing rancidity and serve as stabilizers.

Other addition agents may include aliphatic amines, or alkylol amines, lead soap, halogenated materials, graphite, phosphoric acid esters, sulfur or sulfur chlorine extreme pressure lubricant bases or sulfur combined into the mineral oil base

stock; modifying agents, such as glycerine, glycols, polyglycols, esters, etc., may also be included.

The invention will be better understood from a consideration of the following examples which are given for illustration only and without intent of limiting the invention to the particular materials and proportions used.

A series of greases was prepared in which slightly different conditions of heating and order of mixing were used, and in which the products were drawn off at different temperatures but the proportions used were all the same.

|                                                  | Per cent by weight |
|--------------------------------------------------|--------------------|
| Oleic acid                                       | 8.00               |
| Hydrated lime                                    | 1.04               |
| Coastal distillate (1130 vis. at 100° F.)        | 18.20              |
| Coastal bright stock (200 secs. vis. at 210° F.) | 72.76              |
|                                                  | 100.00             |

A blend of the Coastal distillate and the Coastal bright stock in the proportions given above, has a viscosity of about 150-160 seconds Saybolt at 210° F. This grease has a free acidity of 0.66%.

As will appear from the table herebelow, in each case the oleic acid was dissolved in some of the oil and the hydrated lime was suspended in some of the oil and then the resulting solution and suspension were mixed together to effect the saponification reaction, in some cases the acid solution being put into the kettle first and consequently heated first before heating the lime suspension, and in other cases the reverse procedure being used, namely, heating the lime suspension first and then adding the acid solution to it. This latter order of mixing is preferred as it prevents objectionable settling of the lime suspension, since the agitator in the mixing kettle can be kept stirring during the entire procedure. It will also be noted that in some tests part of the oil was reserved for quenching the reaction mixture, i. e., for cooling the mixture from the reaction temperature down to a temperature substantially below that. In all cases where the temperature of drawing was below the temperature of working, the grease mixture was stirred during the cooling, but after the grease was drawn into cans or other suitable containers for storage or shipment, it was not subjected to any further mechanical working until it was cooled down to the room temperature and also ready to be subjected to the penetration tests (made according to the regular A. S. T. M. method).

Table

|                                     | Test No. |         |     |            |             |            |
|-------------------------------------|----------|---------|-----|------------|-------------|------------|
|                                     | 1        | 2       | 3   | 4          | 5           | 6          |
| Amt. of oil with oleic acid         |          |         |     |            |             |            |
| Distillate                          | 1st      | 1st     |     | 2d         |             | 2d         |
| Bright stock                        | 100      | 67      |     | 100        |             | 100        |
| 2d                                  | 2d       | 2d      |     | 1st        |             | 1st        |
| Amt. of oil with hyd. lime          | 100      |         | 22  | Same as #2 | 67          | Same as #4 |
| Distillate                          |          |         |     |            |             |            |
| Bright stock                        |          |         |     |            |             |            |
| Oil for Quenching:                  |          |         |     |            |             |            |
| Distillate                          |          | 100     |     |            |             |            |
| Bright stock                        |          | 11      |     | 33         |             |            |
| Temp. (max.) of mixing (°F.)        | 180      | 180     |     | 175        |             | 190        |
| Temp. drawing                       | 160      | 150-160 | 130 | 160        | 130         | 190        |
| Penetration unworked                | 390      | 328     | 380 | 322        | 380-400     | 165        |
| Penetration worked                  | 294      | 296     | 295 | 283        | 320         | 285        |
| Penetration difference <sup>1</sup> | -96      | -32     | -85 | -39        | -70 (aver.) | 100        |

<sup>1</sup> Minus sign means decrease in penetration.

Test No. 6 represents the type of penetration characteristics obtained in prior art products where usually the penetration of the greases increased with working at room temperature. In all the other tests, i. e., Nos. 1 to 5, where the product had been cooled down from the reaction temperature substantially, before drawing, the resulting greases decreased in penetration upon working, this decrease ranging in extent from about 20-95 units.

In order to emphasize more clearly the surprising results of the present invention, the penetration figures of tests 4, 5, and 6 are set forth graphically in the accompanying drawing in which the A. S. T. M. penetration (on the vertical axis is plotted against drawing temperature on the horizontal axis). This drawing shows clearly that when the grease is drawn at 190° F. the unworked penetration is substantially lower than the worked penetration, but that when the same type of grease is cooled down to 160° F. or further on down to 130° F. (with stirring) before drawing, the resultant product when cooled down to room temperature has an unworked penetration which is substantially higher than the worked penetration. The chart also shows that the graphs for the worked and unworked penetrations cross each other at a temperature of about 173° F. or 174° F. When this type of grease, i. e. made at 175° F. or higher, is stirred and cooled down to about 174° F. and drawn at this temperature the resulting grease will have substantially the same unworked and worked penetrations, and when cooled further before drawing the unworked penetration becomes increasingly higher and the difference between unworked and worked penetrations becomes increasingly greater.

As discussed previously, the greases of this invention are particularly suitable for cam and automobile shackle lubrication and many other purposes where it is desired that the grease should not become thinner during working and especially where it is desired that the grease should even become harder upon working.

It is not intended that this invention be limited to any theory as to the mechanism of the operation of the present invention nor to the materials and purposes which have been given merely as illustrative, but only by the appended claims by which it is intended to claim all novelty inherent in the invention as broadly as the prior art permits.

We claim:

1. A lime soap grease comprising a major proportion of mineral oil base stock and a minor proportion of lime soap made from proportions of a fatty acid having more than 10 carbon atoms and lime corresponding approximately to 8.00% of oleic acid and 1.04% of hydrated lime, and made at a saponification temperature of 150° to 200° F. and drawn at a temperature below 175° F., at least 15° F. below the saponification temperature, said grease having an A. S. T. M. worked penetration of at least 30 units lower than unworked.

2. A grease according to claim 1 made from an oil base stock having a viscosity greater than about 50 seconds Saybolt at 210° F.

3. A grease according to claim 1 made from an essentially naphthenic oil.

4. A grease according to claim 1 made from oleic acid.

5. Grease according to claim 1 also containing a small amount of soap selected from the group consisting of soda soap and aluminum soap.

6. A grease according to claim 1 made from an essentially mixed base hydrocarbon oil base stock having a viscosity of about 100-200 seconds Saybolt at 210° F., and comprising about 2% to 25% of a lime fatty acid soap.

7. Grease according to claim 1 made from a non-paraffinic oil of the range of bright stock and cylinder oil.

8. A grease according to claim 1 made at a temperature at below 210° F. and, after stirring and cooling, finished and drawn at a temperature between about 160° F. to 120° F.

9. A lime soap grease made from approximately the following proportions of materials:

|                                                      | Per cent |
|------------------------------------------------------|----------|
| Oleic acid                                           | 8        |
| Hydrated lime                                        | 1.04     |
| Coastal oil distillate of about 1130 vis. at 100° F. | 18.20    |
| Bright stock of about 200 secs. vis. at 210° F.      | 72.76    |

the said grease having been manufactured at a temperature of about 175° F. to 190° F., and, after stirring and cooling, drawn at a temperature between about 160° F. to 120° F., and the said grease having the property of becoming harder when worked or passed through grease dispensing equipment at normal temperatures.

10. A lubricating grease made from approximately the following proportions of materials:

|                         | Per cent |
|-------------------------|----------|
| Oleic acid              | 8.00     |
| Hydrated lime           | 1.04     |
| Mineral lubricating oil | 90.96    |

said grease being made at a saponification temperature of about 175° to about 210° F. and drawn at a temperature at least as low as 160° F.

11. The process of making a lime soap grease with an oil base stock having a viscosity greater than about 55 seconds Saybolt at 210° F., which comprises making a lime soap in the presence of at least part of the oil using proportions of acid and lime corresponding substantially to 8.00% oleic acid and 1.04% hydrated lime, at a temperature of about 175°-200° F., and drawing the grease at a temperature below about 175° F., whereby a grease is obtained having an A. S. T. M. worked penetration of at least 30 units lower than unworked.

12. The process of making a lime soap grease which comprises mixing a fatty acid with part of the oil to be used, mixing hydrated lime with another part of the oil, using proportions of acid and lime corresponding substantially to 8.00% oleic acid and 1.04% hydrated lime, and reacting the two resultant mixtures at a temperature at least as high as 150° F. but not above 210° F., stirring or pumping the grease-making ingredients and cooling to and drawing at a temperature below 175° F. at least 15° F. below the saponification temperature used.

13. Process according to claim 12 in which a part of the oil is used to quench the grease from the reaction temperature down to the drawing temperature.

14. The process of making a lime soap lubricating grease which comprises making a suspension of hydrated lime in a Coastal oil distillate, stirring and heating this suspension to a temperature of about 175° F. to 200° F., adding thereto a solution of oleic acid in a Coastal oil distillate, using proportions of acid and lime corresponding substantially to 8.00% oleic acid and 1.04% hydrated lime, maintaining the tempera-

ture of the mixture at a temperature between 150° F. to 200° F. until the saponification reaction is complete, adding additional Coastal oil, with stirring, to cool the mixture, and drawing the resulting grease at a temperature between about 160° F. to 120° F., the different fractions of oil used having such consistencies that a blend of

all of the oil would have a viscosity of about 100 to 200 seconds Saybolt at 210° F., and said grease having an A. S. T. M. worked penetration of at least 30 units lower than unworked.

ARNOLD J. MORWAY.  
JOHN C. ZIMMER.